

## UNITED STATES PATENT OFFICE.

FRANK A. FAHRENWALD, OF CLEVELAND HEIGHTS, OHIO.

## SHELL OR CARTRIDGE CASE.

No Drawing.

Application filed February 26, 1920. Serial No. 361,394.

*To all whom it may concern:*

Be it known that I, FRANK A. FAHRENWALD, a citizen of the United States, residing at Cleveland Heights, in the county of 5 Cuyahoga and State of Ohio, have invented a certain new and useful Improvement in Shell or Cartridge Cases, of which the following is a full, clear, and exact description.

This invention relates to an improvement 10 in cartridge cases and primers for use in ordnance or the manufacture of sporting or military cartridges. In small sized arms the loading unit is called a "cartridge" and consists of a powder container having a 15 charge of propellant therein, a projectile or bullet in one end and a fulminating charge in the other end; in the smallest cartridges the latter is frequently spread over the bottom of the powder container and penetrates 20 into a fold around the base of the same, being exploded by a blow upon the rim, whence arises the name "rim-fire cartridges"; in the larger sizes the fulminate 25 is contained in a separate member called the "primer," used in the base of the powder container generally at the center, wherefore these are called "center-fire cartridges." In these small sized units, the powder container is called a "shell" and has hitherto 30 been made of copper for the smallest arms, brass for the medium and high powered rifles, and of brass and paper for shot-guns. In small ordnance the loading unit ordinarily employed is of the same description 35 as the "center fire" rifle cartridge, except that the term "shell" is applied to the projectile instead of to the powder container, the latter being ordinarily made of brass. In large ordnance, the projectile is handled 40 and inserted independently of the propellant, the latter being ordinarily contained in fabric bags.

The present invention relates to the powder-container (and also to the primer in 45 case one is used) and to this part or combination of parts I apply the term "cartridge case," intending thereby to include both powder container and primer (in cases where the latter is a separate part) regard- 50 less of the size of arm and regardless of whether one bullet or many be employed and whether the same be affixed in or to such cartridge case or be handled separately. The metals and alloys heretofore 55 used for these parts suffer the defects of great weight, high intrinsic value, and sus-

ceptibility to corrosion. The first of these serves to limit unduly the labor of carrying an adequate supply of ammunition, the second renders the ammunition unduly expensive, and the third impedes or prevents re-loading and sometimes renders difficult the extraction of the cartridge case after firing. The objects of my invention are the provision of a cartridge case which is not affected by ordinary atmospheric influences, by powder residues, or by salt solutions encountered in actual practice such as sea water and perspiration; the provision of a cartridge casing of less weight than the ordinary one of brass or copper, and which is of lower intrinsic value; the provision of a shell material whose cost of manufacture, due to the greater ductility of the alloy and the lower temperatures required for working and annealing during drawing operations, will also be substantially lower; while further objects and advantages of the invention will appear as the description 60 proceeds.

The essence of my invention consists in the employment of alloys composed chiefly of aluminum together with smaller quantities of hardening and toughening materials, principally copper and magnesium. Silicon has a desirable effect when present to not over about  $\frac{1}{2}\%$ , and the hardness and elasticity of the alloy are greatly increased by the addition of small amounts of manganese, chromium or iron group metals. 65 The use of zinc or similar metals, however, renders the alloy so easily fusible and so lowers the annealing temperature that its use is not desirable. Iron, manganese, or nickel may be employed up to about two per 70 cent, although I prefer to keep them below about one per cent. I have added copper up to about eight per cent and magnesium up to about twelve per cent without causing the alloy to become so hard that it could 75 not be worked into the desired shapes. I prefer, however, to keep the copper between about one-half per cent and six per cent and the magnesium below about six per cent, and the more refractory metals below 80 about 1.5 per cent. I have found that it is practically impossible to add more than about fifteen per cent of all alloying constituents combined without destroying the properties of these aluminum alloys for cartridge case purposes, other elements such as 85 molybdenum, tungsten, vanadium, titani-

um, etc., may be used in small amounts without detriment and even with beneficial results, but the advantages accompanying their use are more than outweighed by their greater cost. The limits of feasible composition of my alloy are between about eighty-five to ninety-nine per cent of aluminum with one to fifteen per cent of the other substances named, one per cent of hardening substance being reasonably satisfactory in the smaller size shells when the same consists of one or more of the substances, magnesium, silicon, iron, manganese, nickel, molybdenum, tungsten, vanadium, or titanium and eighty-five per cent of aluminum alloyed with eight per cent of magnesium, five per cent of copper, two per cent manganese copper, iron and silicon or iron-group metals, etc. It is desirable, however, to employ limits less extensive than these, especially the upper limits of hardening materials. My preferred alloy consists of:

|                                        |       |
|----------------------------------------|-------|
| Aluminum                               | 95.5% |
| Copper                                 | 1.5%  |
| Magnesium                              | 2.0%  |
| Manganese                              | 0.4%  |
| Iron and silicon or iron-group metals. | 0.6%  |

30 Different types of cartridge cases require different grades of alloys, however, so it is necessary to vary the composition to meet these requirements. It is essential, for instance, to employ a much softer alloy for 35 rim-fire cartridges than for those which are equipped with a cap. In this case the fulminate is fired by being compressed between inner surfaces of the fold which forms the head of the shell. When as in this case, a 40 softer and tougher alloy is required, the amount of hardening and toughening constituents may be materially reduced. A similar effect may be brought about by suitably annealing after all drawing and 45 forming operations are completed.

For certain sporting and military cartridges, however, it is necessary to increase the amount of hardening and toughening constituents, and to form the shell with 50 the least required amount of annealing in order to produce a shell in which the material has been subjected to the greatest possible amount of cold work with its resulting high values for tensile strength and elasticity.

It is also possible to improve the qualities of these alloys by a suitable heat treatment, and for certain requirements the properties so produced are essential. This 55 treatment consists in subjecting the alloy to a temperature between 450° to 550° and

then quenching in some suitable medium at a temperature which varies with the grade of alloy.

In the cold worked condition some of the 65 above described alloys possess a tensile strength upward of seventy thousand pounds per square inch which is far above that required in most cartridge cases.

The above described alloys are particularly adapted to the manufacture of rifle and pistol cartridges from the small twenty-two caliber to the more powerful high velocity type, although shotgun shells and larger cases for ordnance may be made of this alloy with great satisfaction. Owing to the very low specific weight of aluminum, a given case of this material costs less than a similar case of brass despite the higher 80 cost of aluminum per pound. Likewise, the extremely light weight of the alloy decreases the total weight of the loaded cartridge to a remarkable extent, in many instances connected with military cartridges 85 as much as one-third, thereby enabling a soldier to carry a fifty per cent increased supply of ammunition with the same labor. Furthermore, this material remains bright and untarnished almost indefinitely when subjected to salt solutions, atmospheric conditions, or even to powder gases and residues, as a result of which it neither becomes fouled in carrying or sticks in the 90 firing chamber. Its elasticity is such as to cause it to return to its original size after each firing notwithstanding the instantaneous expansion by the powder gases, thus avoiding extraction difficulties and rendering reloading possible. Its low cost renders 95 it feasible for use in shot gun shells and in powder containers for heavy ordnance. It is without chemical action on propellants or fulminates. It can be drawn and worked with the greatest ease. In the case of certain extremely high-velocity sporting or 100 military cartridges of the so-called "rimless" type, I have found it advisable to support the base of the shell of the case with a cup or ring of some harder or stiffer material such as steel or bronze to prevent 105 crushing and I lay claim to such composite cartridge cases as a part of my invention 110 which fall within the annexed claim.

Having thus described my invention, what I claim is:

A cartridge case made from an alloy containing approximately, 95.5% aluminum, 1.5% copper, 2.0% magnesium, 1.0% a metal adjacent to iron in the periodic table.

In testimony whereof, I hereunto affix my 120 signature.

FRANK A. FAHRENWALD.